

# UNITED STATES PATENT OFFICE.

LOUIS JUNIOR, OF BELLEVILLE, ILLINOIS.

## COMPOSITION FOR IMPROVING LACE-LEATHER.

SPECIFICATION forming part of Letters Patent No. 253,210, dated February 7, 1882.

Application filed August 8, 1881. (No specimens.)

*To all whom it may concern:*

Be it known that I, LOUIS JUNIOR, a citizen of the United States, residing at Belleville, in the county of St. Clair and State of Illinois, have invented a new and useful composition of matter to be used in the process of tanning to make lace-leather strong, elastic, and durable, of which composition the following is a specification.

10 My composition consists of the following ingredients, combined in the proportions stated, viz: for every ten pounds of hide—pure water, five gallons; alum, one pound; sal-soda, four ounces; common salt, four ounces; wheat-bran, 15 (or other bran,) four ounces. Of these ingredients the crystalline salts should be thoroughly dissolved and mingled by agitation with the bran.

In using the above-described composition 20 the hides must go through the following processes, viz:

First. Soak the hides in fresh water for twenty-four hours.

Second. Soak the hides in freshly-slaked-lime water as long as necessary to make the hair removable by scraping.

Third. Put the unhaired hides into fresh lime-water once more for two days.

Fourth. Scrape off all fleshy parts on the 30 side; then soak the hides in fresh water to free them from all lime.

Fifth. Then rub the hides with a "slick-stone," in order to smooth or burnish them and to squeeze out all impurities.

35 Sixth. Soak the hides for about twelve hours in warm water, containing one pound of wheat-bran and one-half pound of a ferment to every five gallons of water, until the hides cease to swell and all lime is neutralized.

Seventh. Then squeeze them well with the scrape-iron.

Eighth. Immerse the hides in the above and first-described composition, in which they are to remain for from twelve to twenty-four hours, 45 till the hides are well penetrated (saturated) by the compound; then take them out and hang them up to dry. (The application of this solution in tanning in connection with my other treatment of the hides has the effect of preserving the whole natural strength of the same, which is possible only in the absence of free acids.)

Ninth. Now work them well on the stretch-

bench and split them evenly on the splitting-machine.

Tenth. Rub into the hides a mixture of about three pounds of lard-oil and one pound of tallow, and let dry well. (The proportions of lard-oil and tallow change a little, according to the temperature of the season, so that more tallow and less oil is used in summer than in winter. The exact proportions cannot be prescribed.)

Eleventh. Soak in rain-water containing bran, and in this wet state stretch the hides 65 well on the stretch-bench.

Twelfth. Now shave them as clean as possible on the flesh side, and especially carefully on the grain side, in order to remove the whole grain, which removal produces the elasticity 70 which distinguishes my lace-leather from any other and prevents the liability of cracking.

Thirteenth. Then, finally, rub into the hides a mixture of one and one-half pound of lard-oil, one-half pound of tallow, and one-eighth pound 75 of fine flour for every ten pounds of hide, (which process helps to produce smoothness and durability of the leather,) let them dry, then stretch and smooth them well with a wooden stretcher, and now the hides are ready for use.

I consider it a main feature of my process or style of tanning that there are no free acids used, and that, as a consequence of that fact, together with the other treatment, the hides keep their full natural strength, smoothness, 85 and elasticity.

I am aware that some, perhaps all, the ingredients constituting the alum composition (the only one I claim) are used in tanning; but I am not aware that all of these ingredients 90 have been used together and in the proportions stated for the same purpose.

I do not claim the process described; but I reserve the right to make it the subject of a future application.

What I claim, and wish to secure by Letters Patent of the United States, is—

The herein-described composition of matter, consisting of water, alum, sal-soda, common salt, and bran, in the proportions and for the 100 purpose stated.

LOUIS JUNIOR.

Witnesses:

JOSEPH TROLL,  
FREDERICK BECHTOLD.